

## 1

3,730,892

**PRODUCTION OF POLYESTERS**

Robert Moore Marshall, Chester, and Kimon Constantine Dardoufas, Richmond, Va., assignors to Allied Chemical Corporation, New York, N.Y.  
No Drawing. Filed Mar. 22, 1971, Ser. No. 126,963

Int. Cl. D06m 13/38

U.S. Cl. 252—8.75

9 Claims

**ABSTRACT OF THE DISCLOSURE**

An improved multifilament polyethylene terephthalate yarn and process for producing said yarn, said yarn being combined with a compatible fiber finish composition of hexadecyl (isocetyl) stearate, coconut oil or mineral oil; glycerol monooleate; decaglycerol tetraoleate; polyoxyethylene tall oil fatty acid; sulfonated glycerol trioleate; polyoxyethylene tallow amine; 4,4'-thiobis (6-tert-butyl-m-cresol); and a silane having the structural formula


 wherein  $n=2$  to 5.

**BACKGROUND OF THE INVENTION**

This invention relates to multifilament yarns and particularly to improved multifilament polyethylene terephthalate yarns for industrial uses. More particularly, it relates to an improved multifilament polyethylene terephthalate yarn and a new fiber finishing process for polyethylene terephthalate yarns in which novel fiber finish compositions are applied to said yarns. Still more particularly, it relates to a fiber finish composition designed specifically for subsequent single dip tire cord processing for polyethylene terephthalate yarns.

Many fiber finish compositions are known. Some are quite specific in composition and relate to specific type fibers. Small changes in fiber finish composition frequently result in tremendous improvements in not only processing but also in end use of the fiber. One problem is that two chemical dip treatments are currently required for polyester tire cord in order to obtain fiber to rubber adhesion required in the use of fiber in tires.

This invention provides a new approach to improve the dual finish system. It provides a method by which reactive adhesion promoting chemicals are applied to the yarn after the draw zone thus avoiding the critical process conditions. This invention also allows the elimination of the heretofore isocyanate dip in cord processing. Such, it is believed will make a significant contribution to this highly sophisticated art.

Accordingly, a prime object of this invention is to provide an improved polyester yarn and an improved fiber finishing process for polyethylene terephthalate yarns in which novel fiber finish compositions are applied to said yarns. Other objects will be apparent from time to time in the following specification.

**SUMMARY OF THE INVENTION**

These and other objects are obtained in accordance with one mode of the present invention by providing polyethylene terephthalate filaments having incorporated therein from about 0.5 to about 1.4 weight percent based on the weight of the yarn of a compatible fiber finish composition of about 45 to 50 parts by weight of hexadecyl (isocetyl) stearate; about 4 to 6 parts by weight of glycerol monooleate; about 3.5 to 5.5 parts by weight of decaglycerol tetraoleate; about 5.5 to 8.1 parts by weight

## 2

of polyoxyethylene tall oil fatty acid; about 8.0 to 10.0 parts by weight sulfonated glycerol trioleate; about 2.0 to 3.0 parts by weight polyoxyethylene tallow amine; about 1.0 to 2.0 parts by weight 4,4'-thiobis(6-tert-butyl-m-cresol); and about 5 to 30 parts by weight of a silane having the structural formula


 wherein  $n=2$  to 5.

Another mode of this invention is attained by providing polyethylene terephthalate filaments having incorporated therein from about 0.5 to about 1.4 weight percent based on the weight of the yarn of a compatible fiber finish composition of about 3 to 5 parts by weight of glycerol monooleate, about 3 to 5 parts by weight of decaglycerol tetraoleate, about 4 to 8 parts by weight of polyoxyethylene tall oil fatty acid, about 6 to 10 parts by weight of sulfonated glycerol trioleate, about 3 to 5 parts by weight of polyoxyethylene tallow amine, about 1.0 to 2.0 parts by weight 4,4'-thiobis(6-tert-butyl-m-cresol), about 10 to 30 parts by weight of a silane having the structural formula



wherein  $n=2$  to 5, and 49 to about 55 parts by weight coconut oil.

Still another mode of this invention is attained by providing polyethylene terephthalate filaments having incorporated therein from about 0.5 to about 1.4 weight percent based on the weight of the yarn of a compatible fiber finish composition of about 3 to 5 parts by weight of glycerol monooleate, about 8 to 12 parts by weight of decaglycerol tetraoleate, about 6 to 12 parts by weight of polyoxyethylene tall oil fatty acid, about 10 to 14 parts by weight of sulfonated glycerol trioleate, about 1 to .3 parts by weight of 4,4'-thiobis(6-tert-butyl-m-cresol), about 5 to 30 parts by weight of a silane having the structural formula



wherein  $n=2$  to 5, and about 40 to 48 parts by weight mineral oil.

One of the great advantages of this invention lies in the fact that the fiber finish composition is applied to the filaments after normal processing or preparation thereby avoiding many of the processing problems, such as, heat losses from vaporization of volatile components in fiber finishing components, particularly using aqueous systems as well as others.

Another real advantage of this invention is that it eliminates the need for the isocyanate dip in cord processing.

These and other advantages can more fully be appreciated when viewed in light of the following examples along with the discussion in the specification. These examples illustrate in Tables I-IV applicants' invention and advantages. These tables further illustrate the interrelationship of these fiber finish compositions with fiber performance in relation to double versus single dip adhesion as well as confirmation of these results in tire cord physical properties. These examples are illustrative only and are not to be construed as limitative.

TABLE I.—FINISH COMPOSITION (PARTS BY WEIGHT)

| Finish components                             | Finish identities |    |    |    |    |    |    |        |        |        |        |        |        |        | Function |                      |                     |
|-----------------------------------------------|-------------------|----|----|----|----|----|----|--------|--------|--------|--------|--------|--------|--------|----------|----------------------|---------------------|
|                                               | A                 | B  | C  | D  | E  | F  | G  | H      | I      | J      | K      | M      | N      | O      | P        |                      |                     |
| Hexadecyl stearate.....                       | 63                | 56 | 52 | 38 |    |    |    | 54     | 54     | 52     | 49     | 52     | 49     | 51     |          | Lubricant.           |                     |
| Glycerol monoleate.....                       | 6                 | 5  | 4  | 3  | 4  | 4  |    | 5      | 5      | 4      | 4      | 4      | 4      | 4      |          | Emulsifier.          |                     |
| Decaglycerol tetraoleate.....                 | 5                 | 4  | 4  | 3  | 4  | 10 |    | 4      | 4      | 4      | 4      | 4      | 4      | 4      |          | Do.                  |                     |
| Poo (6) tall oil fatty acid.....              | 8                 | 7  | 6  | 3  | 6  | 8  |    | 7      | 7      | 6      | 5      | 6      | 5      | 6      |          | Do.                  |                     |
| Sulfated glycerol trioleate.....              | 12                | 10 | 8  | 5  | 8  | 12 |    | 10     | 10     | 8      | 7      | 8      | 7      | 8      |          | Antistat emulsifier. |                     |
| Poo (20) tallow amine.....                    | 4                 | 4  | 4  | 2  | 4  |    |    | 3      | 3      | 4      | 4      | 4      | 4      | 4      |          | Do.                  |                     |
| 4,4' thiobis(6-tert-butyl-m-cresol).....      | 2                 | 2  | 2  | 1  | 2  | 2  | 2  | 2      | 2      | 2      | 2      | 2      | 2      | 2      | 2        | Anti-oxidant.        |                     |
| Gamma glycidoxypropyl trimethoxysilane.....   | ---               | 12 | 20 | 45 | 20 | 20 | 20 |        |        |        |        |        |        |        |          | Adhesion activator.  |                     |
| Coconut oil.....                              |                   |    |    |    |    |    | 52 |        |        |        |        |        |        |        |          | Lubricant.           |                     |
| Mineral oil (200 SUS).....                    |                   |    |    |    |    |    | 44 |        |        |        |        |        |        |        |          | Do.                  |                     |
| Triethylenglycol dipelargonate.....           |                   |    |    |    |    |    | 78 |        |        |        |        |        |        |        |          | Do.                  |                     |
| Other adhesion activators (see Table II)..... |                   |    |    |    |    |    |    | 15 (1) | 15 (2) | 18 (3) | 18 (5) | 20 (7) | 17 (8) | 15 (9) | 15 (10)  | 18 (11)              | Adhesion activator. |
| Assistants (Table II).....                    |                   |    |    |    |    |    |    |        |        | 2 (4)  | 7 (6)  |        | 8 (6)  | 6 (6)  | 5 (6)    | 7 (6)                | Do.                 |

TABLE II

## Other adhesion activators and assistants

- (1) Gamma methacrylicpropyl trimethoxysilane
- (2) Beta 3,4(epoxycyclohexyl) ethyltrimethoxysilane
- (3) Dimethyl polysiloxane
- (4) Aluminum stearate
- (5) Triallylisocyanurate
- (6) Eponite 100 polyepoxide
- (7) Triglycidylisocyanurate
- (8) Polyethylene imine
- (9) Tris(2-hydroxyethyl) isocyanurate
- (10) Bis phenol adduct of methylene bis(4-phenyl isocyanate)
- (11) Tolyene 2,4 diisocyanate

TABLE V

## Yarn to yarn friction of overfinish PET tire yarn

| 25 | Finish identity                         | Yarn to yarn friction in gm. <sup>1</sup> |                         |
|----|-----------------------------------------|-------------------------------------------|-------------------------|
|    |                                         | No yarn/finish                            | Yarn/finish "A" control |
|    | No yarn/finish                          | 160-621                                   |                         |
|    | Yarn/finish "A" control                 | 240-625                                   |                         |
|    | Yarn/finish "C," 20% Additive OWC       | 395                                       |                         |
|    | Yarn/finish "B," 12% Additive OWC       | 388                                       |                         |
| 30 | Yarn/finish "H," 15% other Additive OWC | 250-477                                   |                         |

<sup>1</sup> 1200 grams pretension, 360° angle.

Table I discloses various examples of the compatible fiber finish composition in accordance with this invention in parts by weight compared with a control Example A.

TABLE III.—SCREENING TRIAL SINGLE DIP ADHESION RESULTS IN PERCENT OF DOUBLE DIP CONTROL

| Double dip "A" control                                       | Finish identity |      |     |      |      |      |        |      |     |      |      |     |     |     | NON AQ | NON AQ |
|--------------------------------------------------------------|-----------------|------|-----|------|------|------|--------|------|-----|------|------|-----|-----|-----|--------|--------|
|                                                              | B               | C    | D   | E    | F    | G    | H      | I    | J   | K    | L    | M   | N   | O   |        |        |
|                                                              | AQ              | AQ   | AQ  | AQ   | AQ   | AQ   | NON AQ | AQ   | AQ  | AQ   | AQ   | AQ  | AQ  | AQ  |        |        |
| Percent oil on yarn.....                                     | 1.11            | 1.06 | .95 | 1.01 | 1.66 | 1.12 | 1.38   | 1.01 | .93 | 10.7 | 1.07 | .87 | .89 | .76 | 1.07   | 1.83   |
| Percent additive on yarn.....                                | .11             | .18  | .38 | .18  | .19  | .24  | .13    | .12  | .18 | .23  | .12  | .15 | .15 | .19 | .33    | .28    |
| Adhesion $\frac{3}{8}$ " cold percent of double dip "A"..... | 100             | 93   | 93  | 90   | 88   | 84   | 68     | 36   | 63  | 39   | 70   | 67  | 78  | 59  | 73     | 58     |
| Adhesion $\frac{3}{8}$ " hot percent of double dip "A".....  | 100             | 98   | 93  | 92   | 86   | 83   | 58     | 32   | 57  | 41   | 72   | 53  | 72  | 55  | 69     | 50     |

TABLE IV.—CONFIRMATION AND TIRE CORD PROPERTIES TRIAL

|                                                              | Finish identity |      |      |      |  |
|--------------------------------------------------------------|-----------------|------|------|------|--|
|                                                              | D               | C    | B    | A    |  |
| Percent oil on yarn.....                                     | 1.01            | 1.06 | 1.06 | 1.08 |  |
| Percent additive on yarn.....                                | .38             | .21  | .11  |      |  |
| Yarn:                                                        |                 |      |      |      |  |
| Breaking strength in lbs.....                                | 26.2            | 26.1 | 26.3 | 26.8 |  |
| Percent elongation at break.....                             | 15.0            | 15.1 | 14.4 | 14.4 |  |
| Greige cord:                                                 |                 |      |      |      |  |
| Breaking strength in lbs.....                                | 67.8            | 68.3 | 68.4 | 70.1 |  |
| Percent elongation at break.....                             | 21.0            | 21.0 | 20.2 | 20.4 |  |
| Translational efficiency, percent.....                       | 86              | 87   | 87   | 87   |  |
| Thermal stability percent retained strength.....             | 76              | 73   | 67   | 70   |  |
| Dipped tensilized cord.....                                  | (1)             | (2)  | (3)  | (4)  |  |
| Breaking strength in lbs.....                                | 62.3            | 63.2 | 63.7 | 63.9 |  |
| Percent elongation at break.....                             | 16.4            | 16.9 | 15.7 | 14.8 |  |
| Translational efficiency, percent.....                       | 79              | 81   | 81   | 80   |  |
| Thermal stability—percent retained strength.....             | 76              | 79   | 80   | 82   |  |
| Extension compression fatigue percent retained strength..... | 89              | 73   | 93   | 84   |  |
| Adhesion $\frac{3}{8}$ " hot lbs.....                        | 26              | 26   | 27   | 29   |  |
| Adhesion $\frac{3}{8}$ " cold lbs.....                       | 40              | 42   | 43   | 43   |  |

<sup>1</sup> D(RFL) (DIP).<sup>2</sup> C(RFL) (DIP).<sup>3</sup> B(RFL) (DIP).<sup>4</sup> A(BDI and RFL) (DIP).

Table II enumerates other adhesion activators and assistants in accordance with the present invention. Table III illustrates the results of single dip versus heretofore double dip. Example A is shown throughout the examples as the control. Here, in Table III, the results show a single dip of applicants' compatible fiber finish composition with the double dip control (Example A) and the specific parameters of type finish system, percent oil on yarn, percent additive on yarn and the adhesion in both cold and hot situations in percent compared to 100 for the double dip control (Example A).

Table IV then illustrates further confirmation in actual tire cord properties in yarn, greige cord and dipped tensilized cord.

Table V illustrates yarn to yarn friction in accordance with this invention. A pretension of 1200 grams was used along with a 360° angle. The component improves the yarn to yarn frictional properties, thus retaining a good translational efficiency despite the application of an adhesive compound.

The following definitions are used in this invention to define any areas not considered heretofore known or con-

sidered to be part of the prior art. The extension-compression fatigue, sometimes called disk fatigue is used to determine the extension and compression fatigue of textile tire cord. The disk fatigue tester cyclically compresses and extends cord specimens that have been imbedded in cured rubber blocks. After a specified number of compression and extension cycles, the cords are removed from the rubber blocks and tested for tensile strength. The strength of these cords is then compared with that of similar cords that have been cured in rubber but have not been fatigued. The results are then reported in percent strength retained. This method is more specifically described in U.S. Pat. 2,595,069.

We claim:

1. A fiber finish composition consisting of a compatible aqueous emulsion of
- about 45 to 50 parts by weight of isocetyl stearate;
  - about 4 to 6 parts by weight of glycerol monooleate;
  - about 3.5 to 5.5 parts by weight of decaglycerol tetraoleate;
  - about 5.5 to 8.1 parts by weight of polyoxyethylene tall oil fatty acid containing an average of 5 oxyethylene units per mole;
  - about 8.0 to 10.0 parts by weight sulfonated glycerol trioleate;
  - about 2.0 to 3.0 parts by weight polyoxyethylene tallow amine containing an average of 20 oxyethylene units per mole;
  - about 1.0 to 2.0 parts by weight 4,4' thiobis-(6-tert-butyl-m-cresol); and
  - about 5 to 30 parts by weight of a silane having the structural formula



wherein  $n=2$  to 5.

2. A fiber finish composition in accordance with claim 1 wherein the silane is gamma-glycidoxypolypropyltrimethoxysilane.

3. Synthetic filamentary yarn consisting of polyethylene terephthalate filaments which are treated with from about 0.5 to about 1.4 weight percent based on the weight of the yarn of a fiber finish composition consisting of

- about 45 to 50 parts by weight of isocetyl stearate;
- about 4 to 6 parts by weight of glycerol monooleate;
- about 3.5 to 5.5 parts by weight of decaglycerol tetraoleate;
- about 5.5 to 8.1 parts by weight of polyoxyethylene tall oil fatty acid containing an average of 5 oxyethylene units per mole;
- about 8.0 to 10.0 parts by weight sulfonated glycerol trioleate;
- about 2.0 to 3.0 parts by weight polyoxyethylene tallow amine containing an average of 20 oxyethylene units per mole;
- about 1.0 to 2.0 parts by weight 4,4' thiobis-(6-tert-butyl-m-cresol); and
- about 5 to 30 parts by weight of a silane having the structural formula



wherein  $n=2$  to 5.

4. A fiber finish composition consisting of a compatible aqueous emulsion of

- about 3 to 5 parts by weight of glycerol monooleate;
- about 3 to 5 parts by weight of decaglycerol tetraoleate;
- about 4 to 8 parts by weight of polyoxyethylene

5

10

15

20

25

30

35

40

45

50

55

60

65

70

75

tall oil fatty acid containing an average of 5 oxyethylene units per mole;

- about 6 to 10 parts by weight of sulfonated glycerol trioleate;
- about 3 to 5 parts by weight of polyoxyethylene tallow amine containing an average of 20 oxyethylene units per mole;
- about 1.0 to 2.0 parts by weight 4,4' thiobis-(6-tert-butyl-m-cresol);
- about 10 to 30 parts by weight of a silane having the structural formula



wherein  $n=2$  to 5; and

- about 49 to about 55 parts by weight coconut oil.
- A fiber finish composition in accordance with claim 4 wherein the silane is gamma-glycidoxypolypropyltrimethoxysilane.

6. Synthetic filamentary yarn consisting of polyethylene terephthalate filaments which are treated with from about 0.5 to about 1.4 weight percent based on the weight of the yarn of a compatible fiber finish composition consisting of

- about 3 to 5 parts by weight of glycerol monooleate;
- about 3 to 5 parts by weight of decaglycerol tetraoleate;
- about 4 to 8 parts by weight of polyoxyethylene tall oil fatty acid containing an average of 5 oxyethylene units per mole;
- about 6 to 10 parts by weight of sulfonated glycerol trioleate;
- about 3 to 5 parts by weight of polyoxyethylene tallow amine containing an average of 20 oxyethylene units per mole;
- about 1.0 to 2.0 parts by weight 4,4' thiobis-(6-tert-butyl-m-cresol);
- about 10 to 30 parts by weight of a silane having the structural formula



wherein  $n=2$  to 5; and

- about 49 to about 55 parts by weight coconut oil.

7. A fiber finish composition consisting of compatible aqueous emulsion of

- about 3 to 5 parts by weight of glycerol monooleate;
- about 8 to 12 parts by weight of decaglycerol tetraoleate;
- about 6 to 12 parts by weight of polyoxyethylene tall oil fatty acid containing an average of 5 oxyethylene units per mole;
- about 10 to 14 parts by weight of sulfonated glycerol trioleate;
- about 1 to 3 parts by weight of 4,4' thiobis-(6-tert-butyl-m-cresol);
- about 10 to 30 parts by weight of a silane having the structural formula



wherein  $n=2$  to 5; and

- about 40 to 48 parts by weight mineral oil.

8. A fiber finish composition in accordance with claim 7 wherein the silane is gamma-glycidoxypolypropyltrimethoxysilane.

9. Synthetic filamentary yarn consisting of polyethylene terephthalate filaments which are treated with from 0.5

to about 1.4 weight percent based on the weight of the yarn of a fiber finish composition consisting of

- (a) about 3 or 5 parts by weight of glycerol monooleate;
- (b) about 8 to 12 parts by weight of decaglycerol tetraoleate;
- (c) about 6 to 12 parts by weight of polyoxyethylene tall oil fatty acid containing an average of 5 oxyethylene units per mole;
- (d) about 10 to 14 parts by weight of sulfonated glycerol trioleate;
- (e) about 1 to 3 parts by weight of 4,4' thiobis-(6-tert-butyl-m-cresol);
- (f) about 10 to 30 parts by weight of a silane having the structural formula



wherein  $n=2$  to 5; and

- (g) about 40 to 48 parts by weight mineral oil.

#### References Cited

##### UNITED STATES PATENTS

|           |         |                   |             |
|-----------|---------|-------------------|-------------|
| 3,013,966 | 12/1961 | Schiermeier       | 252—8.7     |
| 3,350,345 | 10/1967 | Vanderbilt et al. | 156—110 X   |
| 3,398,045 | 8/1968  | Clayton et al.    | 156—110 X   |
| 3,428,560 | 2/1969  | Olsen             | 252—8.7     |
| 3,503,880 | 3/1970  | McMicken          | 252—8.75    |
| 3,687,721 | 8/1972  | Dardoufas         | 117—138.8 F |

##### OTHER REFERENCES

The Condensed Chemical Dictionary, seventh edition, Pub. 1966 by Reinhold Pub. Corp. of New York, p. 761.

HERBERT B. GUYNN, Primary Examiner

U.S. Cl. X.R.

117—76 T, 138.8 F, 139.5 C.Q.; 156—110 A, 329; 161—206, 231; 252—8.9